

## UNITED STATES PATENT OFFICE

2,387,168

## TREATMENT OF CELLULOSE DERIVATIVE ARTICLES

Robert Wighton Moncrieff and Charles William Sammons, Spondon, near Derby, England, assignors to British Celanese Limited, London, England, a company of Great Britain

No Drawing. Application March 17, 1943, Serial No. 479,492. In Great Britain March 4, 1942

4 Claims. (Cl. 8—132)

This invention is concerned with improvements in the treatment of cellulose derivative articles and particularly in processes for improving the physical properties of yarns, foils and similar articles made of cellulose acetate or other organic derivative of cellulose.

Cellulose acetate yarns, which are the articles with which the present invention is particularly concerned, are produced by dry-spinning a solution of cellulose acetate in acetone and as obtained at the conclusion of the dry-spinning process usually have a tenacity of about 1.1–1.3 grams per denier and an extensibility of about 25%. In order to increase their tenacity they may be subjected to a stretching operation in the presence of a suitable assisting agent, which may be an organic solvent, for example dioxane, or wet steam or hot water. The yarns may be stretched, for instance, to 500 or 1,000% of their original length according to the increase in tenacity which is required and in this manner yarns having a tenacity of 3 or 4 grams per denier or more may be obtained. Yarns made of high viscosity cellulose acetate, e. g. an acetate having a viscosity of 80–100, measured by comparing the rate of flow of a 6% solution of the acetate in acetone with that of glycerine taken as 100, may after stretching have a tenacity as high as 6 grams per denier or even more.

Unfortunately, the increase in tenacity obtained by the stretching operation is almost invariably accompanied by a decrease in extensibility, even with a low degree of stretch. By treating the stretched materials with a shrinking agent, for example a solution of methylene chloride in benzene or toluene, and allowing them to shrink, the extensibility of the yarns may be increased but this increase is accompanied by a decrease in tenacity. For example, it has been found possible in this manner to increase the extension up to 10 or 12% or somewhat more but only at the cost of some of the increase in tenacity produced by the stretching operation.

It has now been discovered that very good results may be obtained as regards improvement in the extensibility of yarns, foils and similar articles made of organic derivatives of cellulose, particularly acetone-soluble cellulose acetate, without causing substantial loss in tenacity, by impregnating them with a medium containing a cyclic ketone, particularly cyclopentanone, without subjecting them to tension sufficient to stretch them. Preferably the treatment is effected under such conditions that a low degree

of shrinkage is effected, e. g. 2–10% of the original length of the materials.

The process of the present invention is of greatest importance in connection with the improvement of the extensibility of yarns and similar articles, for example cords, made of cellulose acetate or other lower fatty acid ester of cellulose, for example cellulose propionate, cellulose butyrate and cellulose acetate-propionate. The materials treated may be made of a cellulose derivative of low, medium or high viscosity. For instance, the process is applicable to the treatment of yarns made of cellulose acetate having a viscosity of 10, 20, 80, 100 or more, determined as described above. The process is most valuable for the treatment of yarns and similar materials which have been stretched, e. g. to 2, 6, 10 or more times their original length, so as to increase their tenacity, for example to 2, 3, 4 or more grams per denier, since, as explained above, such articles usually have an extensibility lower than that desirable for many purposes, for example an extensibility of 6, 8 or 10%. The best results are usually obtained with materials which have been stretched, especially in hot water or wet steam, to between 3 and 5 times their original length. The process is also applicable to the ordinary dry-spun yarns having a tenacity, in the case of yarns made of acetone-soluble cellulose acetate, of about 1.1–1.3 grams per denier, although as such yarns usually have an extensibility of 20–25% or even more, it is not for most purposes necessary to increase it further.

Cyclopentanone has been employed with very good results in the process of the invention, particularly where the materials treated are made of acetone-soluble cellulose acetate or other lower fatty acid ester of cellulose. Other cyclic ketones may however be employed, preferably ones which are liquid at atmospheric temperature, for example, cyclobutanone, cyclohexanone and the methyl-cyclopentanones and cyclohexanones.

The cyclic ketones are preferably employed in solution in organic liquids which themselves have no action on the cellulose derivative forming the basis of the materials under treatment. Such inert liquids include the liquid paraffin hydrocarbons and diethyl ether and other ethers. Mixtures of paraffin hydrocarbons such as are present in petrol, ligroin, benzine and kerosene may be employed.

It has been found that the shrinking effect of the cyclic ketones is greatly enhanced by the presence of small proportions of water. For

example, the shrinking action of a 50% solution of cyclopentanone in petrol on stretched cellulose acetate yarn may be increased 5 to 10 times by the presence of .2-.5% of water in the mixture. It is therefore very important to control the water content, if any, of the shrinking liquid if consistent results are to be obtained. Usually it is preferable to use an anhydrous solution and to dry the yarn or other materials before treatment.

The concentration of the cyclic ketone, the treatment temperature and the time of treatment are all inter-related and a variation in one factor usually involves some variation in one or both of the others in order to obtain the optimum results. When yarns or other articles are treated in batches the treatment may, for example, be carried out using cyclopentanone dissolved in petrol in a concentration of 30-55% at 20-40° C. for about 15-30 minutes. If it is desired to carry out the treatment as a continuous process it is usually preferable to accelerate the action of the cyclic ketone by raising the temperature of the solution employed. For example, yarns made of cellulose acetate may be treated by passing them through a 50% solution of cyclopentanone in petrol at a temperature of 50-60° C., the rate of travel of the yarns and the length of the bath being so arranged that they are in contact with the shrinking liquid for about 30-60 seconds.

It is important that the materials should be thoroughly washed after the treatment in order to remove all traces both of the cyclic ketone and of the diluent employed. Preferably this is effected by washing them first with ether, drying them, giving them a light scour in a very dilute soap solution and then washing them in water, after which they may be dried and conditioned.

After the treatment has been completed the materials may be completely saponified, e. g. with a .6% solution of sodium hydroxide containing 10% of sodium acetate at 60% C. Regenerated cellulose materials having an increased tenacity are thus obtained.

The following examples are given to illustrate the invention.

*Example I*

An ordinary dry-spun yarn made of acetone-soluble cellulose acetate was treated in hank form in a solution containing 38% of cyclopentanone and 62% of petrol by volume for 30 minutes at 25° C. It was then thoroughly washed in ether, dried, given a light scour in .02% soap solution for 5 minutes at 60° C. washed in water, dried and conditioned. The yarn obtained had a substantially increased extensibility and the same tenacity as before the treatment.

*Example II*

A yarn made of acetone-soluble cellulose acetate and stretched in wet steam to 5 times its

original length was treated in hank form in a solution containing 30% of cyclopentanone and 70% petrol by volume at 25° C. for 30 minutes. It was then thoroughly washed as described in the previous example. Its extension was increased by the treatment and there was at the same time a slight increase in tenacity.

An advantage of the cyclic ketones is that they have a low vapour pressure, so that losses through evaporation are not high. Moreover on account of their hydrophile character they are much more easily removed from the materials by scouring than are shrinking agents such as methylene chloride. A particular advantage of cyclopentanone is that the conditions required in order to obtain good results are not so critical as in the case of many shrinking agents.

Having described our invention what we desire to secure by Letters Patent is:

1. Process for the treatment of artificial yarns, foils and similar materials, which comprises impregnating stretched yarns, foils and similar materials having a basis of a lower aliphatic acid ester of cellulose and having an extensibility of 10% or less with an anhydrous medium containing from 30 to 55% by volume of cyclopentanone in the absence of tension sufficient to stretch them and removing the medium from the materials by a washing operation on completion of the treatment.

2. Process according to claim 1 wherein the articles impregnated have been stretched to between 3 and 5 times their original length in the presence of a stretch-assisting agent selected from the group consisting of hot water and wet steam.

3. Process for the treatment of artificial yarns, foils and similar materials, which comprises impregnating stretched yarns and similar materials having a basis of acetone-soluble cellulose acetate and having a tenacity of at least 2 grams per denier and an extensibility of 10% or less with an anhydrous medium containing from 30 to 55% by volume of cyclopentanone in the absence of tension sufficient to stretch them and removing the medium from the materials by a washing operation on completion of the treatment.

4. Process for the treatment of artificial yarns, foils and similar materials, which comprises impregnating stretched yarns, and similar materials having a basis of acetone-soluble cellulose acetate and having a tenacity of at least 2 grams per denier and an extensibility of 10% or less with an anhydrous medium containing from 30 to 55% by volume of cyclopentanone under such conditions that the articles are shrunk by between 2 and 10% of their original length and removing the medium from the materials by a washing operation on completion of the treatment.

ROBERT WIGHTON MONCRIEFF.  
CHARLES WILLIAM SAMMONS.